

## UNITED STATES PATENT OFFICE

JACQUES FRANCOIS MARIE CROLARD, OF WESTMINSTER, ENGLAND, ASSIGNOR TO  
BRITISH-AMERICAN TOBACCO COMPANY, LIMITED, OF LONDON, ENGLAND, A  
BRITISH COMPANY

## MANUFACTURE AND PRODUCTION OF CIGARETTE PAPER

No Drawing. Application filed January 29, 1930, Serial No. 424,454, and in Great Britain April 3, 1929.

My invention relates to improvements in the manufacture and production of paper for cigarettes, and has for its object to provide a cigarette paper which is free from the tendency to become discoloured, stained or 5 spotted by the fixed or volatile oils of the tobacco contained in the cigarette.

According to my invention I incorporate in the cigarette paper a greasy or fatty matter such for example as palmitin, stearin, or the like, the said process of incorporation 10 being effected by precipitation into the pulp of the cigarette paper during the manufacture of the said paper. I have found the best 15 results are obtained by using stearin for the greasy or fatty matter required according to this invention, it being essential in order to obtain the best results to use stearin in the proportion of up to 20 per cent of the pulp 20 employed, giving in the finished paper about 10 per cent of stearin.

The following example illustrates a method of carrying out the invention in practice but the invention is not restricted thereto.

25 *Example*

In a boiler of sufficiently large capacity a mixture composed of: water, 1000 litres; borax, 25 kilograms; and stearin, 50 kilograms, is maintained at boiling for about 30 three hours.

The temperature of the water is raised to boiling point so that the borax will be dissolved and then stearin is added, preferably 35 broken up into small pieces. The boiling should be continued until a few drops of the solution diluted in a large quantity of water give an opalescent solution without any grain, say in about three hours.

40 It is preferred to use indirect heating rather than to allow the steam to enter into the boiler direct. If, however, the latter method be used allowance should be made for the condensation of the steam by reducing 45 the volume of water at the beginning of the operation. The solution is allowed to cool until it reaches a temperature of 40° centigrade, in which state it can be used, but care must be taken that there be no deposit.

50 The solution so obtained is placed either

in the beating machine or in the mixer. If the solution is effected in the beating machine care must be taken when filling the beater to use the minimum amount of water only. If the beater contains 100 kilograms of paste, 55 the quantity of solution to be added would be from 200 to 400 litres according to the intensity of the special effect which it is desired to obtain. The solution should be added about two hours before the end of the beating 60 operation.

In order to precipitate the stearin, aluminium sulphate, calcium chloride or an acid dissolved in hot water is added about an hour before running off the paste contained in the 65 beater according to the quality or kind of the cigarette paper required, for example whether combustible or non-combustible.

Having now particularly described and ascertained the nature of my said invention 70 and in what manner the same is to be performed, I claim:—

1. The manufacture and production of cigarette paper to render the same free from the tendency to become discoloured, stained or 75 spotted after contact with tobacco, by the incorporation with cigarette paper during or after the manufacture of the said paper, of a greasy or fatty matter.

2. In the manufacture of cigarette paper 80 as claimed in claim 1, the use of stearin for the purpose described.

3. The manufacture and production of stain-resisting cigarette paper by the incorporation into the pulp of the cigarette paper 85 during its manufacture a greasy or fatty matter, in proportions up to 20% of the pulp employed.

4. A cigarette paper having a greasy or 90 fatty matter incorporated therein.

In testimony whereof I have signed my name to this specification.

JACQUES FRANCOIS MARIE CROLARD.